

## UNITED STATES PATENT OFFICE

STERNER ST. P. MEEK, OF THE UNITED STATES ARMY, PHILADELPHIA,  
PENNSYLVANIA.

## COMBUSTIBLE

No Drawing.

Application filed September 8, 1925. Serial No. 55,120.

(GRANTED UNDER THE ACT OF MARCH 3, 1863, AS AMENDED APRIL 30, 1928; 370 O. G. 757)

The invention described herein may be manufactured and used by or for the Government for governmental purposes without the payment to me of any royalty thereon.

5 The subject of this invention is a combustible intended, primarily, for use in tracer projectiles for signalling, illuminating or like purposes.

10 The main object of my invention is the imparting of greater visibility, brilliance and luminosity to the combustible.

To this end my invention consists in the use of salts of mercury, either alone, or in combination with other substances. The mercury salts may be used in the form of oxygen carriers, as mercurous oxide, mercuric oxide, mercurous nitrate, etc.; or in the form of a fuel for decreasing the rate of burning of the mixture while at the same time increasing the brilliance by using it in the form of mercuric thiocyanate, mercuric acetate, or mercuric oxalate; or the mercury may be added merely in the form of an inert substance to increase the brilliance, as for example, mercurous chloride, mercuric chloride, mercuric sulphide, etc.

20 As an example of the use of salts of mercury in the form of oxygen carriers the following formulæ are given:

|                                         | Parts |
|-----------------------------------------|-------|
| Strontium nitrate                       | 60    |
| Mercurous nitrate                       | 40    |
| Sodium oxalate                          | 10    |
| Sodium nitrate                          | 8     |
| 35 Magnesium                            | 46    |
| Calcium resinate or a resinous ester    | 28    |
|                                         | Parts |
| Barium nitrate                          | 60    |
| Mercuric oxide                          | 50    |
| Barium oxalate                          | 10    |
| Sodium nitrate                          | 8     |
| Magnesium                               | 34    |
| Aluminum                                | 12    |
| 45 Calcium resinate or a resinous ester | 30    |

The following formula is a typical example of the use of a mercuric salt as a fuel.

|                                      | Parts |
|--------------------------------------|-------|
| Barium nitrate                       | 15    |
| Barium peroxide                      | 12    |
| Calcium resinate or a resinous ester | 12    |
| Magnesium                            | 20    |
| Mercuric thiocyanate                 | 12    |

Of the use of a mercury salt as an inert substance for increasing the brilliance of the combustible the following are examples.

|                                      | Parts |
|--------------------------------------|-------|
| Barium peroxide                      | 20    |
| Barium nitrate                       | 2     |
| Magnesium                            | 7     |
| Calcium resinate or a resinous ester | 3     |
| Mercurous chloride                   | 2     |

and:

|                                      | Parts |
|--------------------------------------|-------|
| Strontium nitrate                    | 100   |
| Strontium oxalate                    | 10    |
| Sodium nitrate                       | 8     |
| Magnesium                            | 34    |
| Aluminum                             | 12    |
| Calcium resinate or a resinous ester | 28    |
| Mercurous chloride                   | 10    |

I claim:

1. A combustible composition including an oxygen carrier, a reducing agent, a binder and a non-fulminating salt of mercury.
2. A combustible including a salt of mercury as an inert substance.
3. A combustible composition including a non-fulminating salt of mercury.
4. A tracer composition comprising salts of mercury.
5. A combustible composition including an inorganic oxidizing ingredient adapted to burn with a characteristic color, a non-fulminating salt of mercury and a reducing agent.
6. A combustible composition including an inorganic oxidizing ingredient adapted to

burn with a characteristic color, a reducing agent and an inert substance comprising a salt of mercury.

7. A combustible composition including an oxygen carrier, a reducing agent, and from 4.95 to 24.5 per cent of a nonfulminating salt of mercury.

STERNER ST. P. MEEK.

**10****15****20****25****30****35****40****45****50****55****60****65**